

1

3,436,214

## COLUMBIUM BASE ALLOY

Mortimer Schussler, Mundelein, Ill., assignor to Union Carbide Corporation, a corporation of New York  
 No Drawing. Continuation-in-part of application Ser. No. 353,252, Mar. 19, 1964. This application Mar. 22, 1967, Ser. No. 625,026

Int. Cl. C22c 27/00

U.S. Cl. 75—174

3 Claims

### ABSTRACT OF THE DISCLOSURE

A columbium base alloy is provided which consists essentially of, by weight, about 5 percent vanadium, about 1 percent zirconium, from about .005 to about .04 percent carbon with the balance being columbium and incidental adventitious impurities. The resultant alloy is both cold rollable and ductile.

This is a continuation-in-part application of Ser. No. 353,252, filed Mar. 19, 1964, now abandoned.

This invention relates to a novel columbium base alloy, and more particularly to an alloy of columbium, vanadium and zirconium which contains beneficial amounts of carbon.

Columbium base alloys in recent years have been proposed for use in applications where severe service conditions are encountered such as exposure to high temperatures, highly corrosive environments and/or unusual amounts of mechanical wear. These conditions are commonly encountered by certain critical components in nuclear power systems and aerospace vehicles.

Unfortunately, only a relatively limited number of well established columbium-base alloys are available commercially, and generally speaking, they are suitable for only a specific use. As a result, whenever a new use or different set of severe service conditions is encountered, an attempt is made to develop a new columbium base alloy having an optimum set of properties for such use.

Illustrative of the present state of the art are the problems encountered with a binary alloy consisting of one percent zirconium balance columbium which has been successively employed in nuclear applications. This particular alloy has acceptable fabricating and welding properties, but certain of the other mechanical and physical, as well as chemical properties are, at best, marginal. With the advent of larger and more efficient nuclear installations, the property requirements of certain components became more critical and the particular alloy under discussion failed to meet the new and more severe requirements. In general, it was discovered that each modification of the alloy for the purpose of improving a particular property to meet a necessary need resulted in an undesirable corresponding effect on another critical property. For example, a modification in the alloy to increase mechanical strength resulted in a reduction in fabricability and weldability. Similarly, an improvement in hardness was accompanied by a reduction in ductility, and an improvement in thermal shock properties was accompanied by a lowered resistance to corrosion.

Accordingly, the principal object of the invention is to provide a columbium base alloy suitable for general industrial use and which is characterized by an optimum combination of physical, mechanical and chemical properties.

Another object of the invention is to provide a columbium base alloy which may be employed in components which will encounter severe service conditions.

A more specific object of the invention is to provide

2

a columbium base alloy which is particularly suitable for use in aerospace and nuclear applications.

An additional object of the invention is to provide a columbium base alloy which is both cold rollable and exceptionally ductile.

The objects of the invention are accomplished by an alloy consisting of, in weight percentages, about 5 percent vanadium, about 1 percent zirconium, between about .005 to about .04 percent carbon with the balance being columbium and adventitious impurities. A higher vanadium content than indicated as within the scope of the invention adversely affects the required high temperature strength properties while excess zirconium content adversely affects the ductility of the alloy.

An unavoidable impurity usually associated with columbium base alloys is tantalum and it may be tolerated up to a maximum of about 5% although it is preferred to be maintained below 1%, if the alloy is to be used in nuclear applications.

Oxygen, nitrogen and hydrogen are harmful to the alloy of the invention and their presence should be kept as low as possible although they can be tolerated in an amount of no more than .03, .02 and .01 percent, respectively.

The total of all other impurities must be kept as low as possible, and in any event should not exceed about 0.1 percent.

The preferred alloy fashioned according to the teachings of the instant invention should contain in excess of 92 weight percent columbium.

With respect to the other undesirable impurities, the following will be of interest.

Elements with relatively low melting points such as titanium and aluminum, if present, tend to weaken the alloy of the invention at high temperatures above about 1800 to 2200° F. Tungsten and molybdenum, if present, in the subject alloy tend to impair its working and welding properties. Further, the inherent high densities of tungsten and molybdenum disturb the desired strength-to-weight ratio of the alloy. Other elements, such as boron, chromium, silicon, iron, cobalt, etc., if present, form secondary phases in the grain boundaries resulting in undesirable working and welding properties. Further, certain elements, especially cobalt, boron, hafnium and tungsten, have a high neutron absorption cross section when compared to the specified elements of the subject alloy (see Table 1) and therefore are harmful if present in the subject alloy, if the alloy is exposed to nuclear radiation.

Table 1.—Neutron absorption cross section, in barns

|           |        |
|-----------|--------|
| Carbon    | 0.0045 |
| Columbium | 1.1    |
| Vanadium  | 5.1    |
| Zirconium | 0.18   |
| Cobalt    | 37.0   |
| Tungsten  | 19.0   |
| Boron     | 750.0  |
| Tantalum  | 21.0   |
| Hafnium   | 115.0  |

The isotope formation of all the elements in the alloy of the invention are very favorable to nuclear thermal reactor exposure. Further, the relatively short "half life" of the radioactive isotopes of these elements and other nuclear properties are also favorable for applications involving nuclear exposure.

Alloys of columbium, vanadium, zirconium and carbon which are within the limits of this invention are alloys that have a low cross section for absorption of thermal neutrons and desirable "half life" characteristics. This is highly desirable for critical components in nuclear applications.

Test results further indicate that the alloy of this invention has good resistance to corrosion in hot water, steam or other similar environments found in thermal reactors.

From the data tabulated below in Table 2, it will be appreciated that the vanadium, zirconium and carbon contents of the alloy of the invention act in a synergistic manner and that the excellent properties of the alloys of the invention are not due merely to the presence of vanadium plus zirconium.

was both cold rollable and also evidenced suitable ductility characteristics.

Alloy 8 was prepared as a 30 pound heat by the well-known consumable electrode arc-melting process in an argon plus helium atmosphere. The alloy was cold reduced to 0.030 inch sheet for further testing and evaluation of the fabricability of the inventive alloys.

Towards this end, Olsen Cup tests and Bend Tests were run on the sheet material which had been subjected

TABLE 2.—EFFECT OF ALLOYING ELEMENTS IN COLUMBIUM ALLOYS

| Alloy No.      | Composition, w/o |      |      | 2,200° F. tensile properties |                                |                 | Hardness Rockwell "B" | Bend ductility, bend radius factor, IT (deg.) |              | Workability to 0.02-inch thick sheet |
|----------------|------------------|------|------|------------------------------|--------------------------------|-----------------|-----------------------|-----------------------------------------------|--------------|--------------------------------------|
|                | V                | Zr   | C    | Yield $\times 1,000$ p.s.i.  | Ultimate $\times 1,000$ p.s.i. | Elong., Percent |                       | Transverse                                    | Longitudinal |                                      |
| 1              | 5                | —    | —    | 19                           | 26                             | 22              | 96                    | 0                                             | 90           | Excellent.                           |
| 2              | —                | 1    | —    | 8                            | 16                             | 14              | 47                    | 180                                           | 180          | Do.                                  |
| 3              | 5                | 1    | —    | 30                           | 31                             | 29              | 92                    | 98                                            | 180          | Do.                                  |
| 4              | 5                | 1    | .1   | —                            | —                              | —               | 98                    | —                                             | —            | Poor.                                |
| 5              | 5                | 1.5  | .1   | —                            | —                              | —               | 100                   | —                                             | —            | Do.                                  |
| 6              | 5                | 3    | —    | —                            | —                              | —               | —                     | —                                             | —            | Do.                                  |
| 7              | 5                | 5    | —    | —                            | —                              | —               | —                     | —                                             | —            | Do.                                  |
| 8 <sup>1</sup> | 5.23             | 1.13 | .005 | 26                           | 27                             | —               | 89                    | 180                                           | 180          | Excellent.                           |

<sup>1</sup> 0.03 inch thick sheet.

Referring to Table 2, Alloy 1 with 5 percent vanadium and Alloy 2 with 1 percent zirconium are both relatively weak alloys at 2200° F. The addition of .1 percent carbon in the alloys tends to embrittle the alloys as noted in Alloys 4 and 5. Alloys 6 and 7 which contain 5 percent vanadium and 3 and 5 percent zirconium, respectively, and which are outside the limits of the invention, are unsuited because they lack sufficient ductility and workability properties. Inventive Alloy 8 which contains a carbon amount which is within the allowable limits illustrates that such an addition of carbon does not embrittle the alloys as does the addition of carbon outside the allowable limits (Alloys 4 and 5). The data in Table 2 clearly show that best results are obtained when the alloy contains about 5 percent vanadium, about 1.0 percent zirconium, less than 0.1 percent carbon and the balance essentially columbium and incidental impurities. Additional data has shown that the carbon content should not exceed .04 weight percent.

Metallographic studies of the alloys listed in Table 2 indicate that the inventive Alloy 8 has a single phase microstructure while Alloys 6 and 7, with higher zirconium contents, appear to have a secondary phase at the grain boundaries. It appears, by correlation, that the microstructure of the alloy influences the working properties of this class of alloys as shown in Table 2.

Five examples of each composition listed in Table 2 (except Alloy 8) were made to obtain average results for the table. Commercially pure columbium, vanadium and zirconium were used in preparing the alloys. The processing steps described herein are within the skills of the present art to produce best results. Each charge was tungsten-arc melted under one-half atmosphere of argon. Each 100-gram button ingot was melted a total of four times and inverted between remelts to achieve alloy homogeneity. The as cast ingots were rolled at 400° F. with 0.01-inch reduction per pass to 0.125-inch thickness. The specimens were then further cold rolled at room temperature to final thicknesses ranging from about 0.10 inch to about 0.01 inch.

The initial reduction step at about 400° F. is, metallurgically, a cold-rolling process because the temperature is below the recrystallization point of the alloy. Through experimentation, it was found that excellent results are obtained when rolling at about 400° F., thus avoiding the harmful effects of hot rolling and eliminating the attendant processing steps required in hot rolling. Considering surface condition and physical-mechanical properties, cold-rolled alloys are superior to hot-rolled alloys. Alloy 3 was readily processed to less than 0.02-inch thickness as described immediately above. However, as noted in Table 2, Alloy 3 did not possess suitable ductility characteristics as evidenced by bend test results. Alloys 4, 5, 6 and 7 were difficult to cold roll, but may be hot rolled at temperatures above about 2000° F. It is to be noted that only Alloy 8

25 to a vacuum anneal of 1 hour at 2100° F. to determine the ductility of the alloy. The Olsen Cup tests showed the alloy to be very ductile and formable; a cup depth of 0.390 inch was obtained under a load of 5120 pounds. The cup test failures were ductile in nature, i.e., deep cups with half-moon type features.

30 Bend test results of 180 degrees over a IT radius were achieved at both room and liquid nitrogen (-321° F.) temperature with the annealed sheet bent both longitudinally and transversely to the final sheet rolling direction.

In addition, two welded bend specimens were prepared by straight line Heliarc<sup>1</sup>, fusion welding of small strips 35 of the annealed sheet in an evacuated dry box. The bend tests were run with the weld bead perpendicular to the bend axis with the root of the weld in compression. Bend angles of 180 and 90 degrees over a IT radius were achieved at room and liquid nitrogen temperature, respectively.

Finally tensile properties over a temperature range of from room temperature to 2400° F. were determined and are reported in Table 3 below.

45 TABLE 3.—TENSILE PROPERTIES OF 0.030-INCH THICK ALLOY NO. 8 SHEET ANNEALED 1 HOUR AT 2,100° F.

| Specimen orientation | Test temperature °F. | Yield stress, 0.2 percent offset, p.s.i. | Ultimate strength, p.s.i. | Elongation percent in 1 inch |
|----------------------|----------------------|------------------------------------------|---------------------------|------------------------------|
| 50                   | Longitudinal...      | 75                                       | 65,000                    | 84,100                       |
|                      | Do.....              | 75                                       | 66,600                    | 85,700                       |
|                      | Traverse.....        | 75                                       | 71,200                    | 90,200                       |
|                      | Do.....              | 75                                       | 73,100                    | 90,200                       |
|                      | Do.....              | 700                                      | 54,800                    | 86,300                       |
|                      | Do.....              | 700                                      | 61,100                    | 87,000                       |
|                      | Do.....              | 1,100                                    | 49,500                    | 87,600                       |
|                      | Do.....              | 1,100                                    | 57,100                    | 101,300                      |
|                      | Longitudinal...      | 2,000                                    | 37,900                    | 43,400                       |
|                      | Do.....              | 2,000                                    | 32,600                    | 39,600                       |
| 55                   | Do.....              | 2,200                                    | 24,500                    | 26,600                       |
|                      | Do.....              | 2,200                                    | 25,600                    | 27,400                       |
|                      | Transverse....       | 2,400                                    | 17,900                    | 18,700                       |
|                      | Do.....              | 2,400                                    | 16,500                    | 18,500                       |

60 As will be appreciated from the foregoing data, the alloy of the subject invention as typified by Alloy 8 in Table 2, has overcome the strength problem associated with the binary columbium-zirconium alloy previously discussed, without impairing producibility.

65 What is claimed is:

1. A cold rollable, ductile alloy consisting essentially of about 5 weight percent of vanadium, about 1 weight percent of zirconium, about .005 weight percent of carbon with the balance being columbium and adventitious impurities.
2. The alloy of claim 1 wherein the weight percent of vanadium is 5.23, the weight percent of zirconium is 1.13 and the weight percent of carbon is .005.

3,436,214

5

3. The alloy of claim 1 wherein the weight percent of columbium is at least 92.

6

3,206,305 9/1965 Begley et al. ----- 75-174  
3,236,638 2/1966 Clark ----- 75-174

References Cited

UNITED STATES PATENTS

3,012,883 12/1961 Allen ----- 75-174  
3,188,207 6/1965 Schussler ----- 75-174

5 Columbium Metallurgy, Interscience Publishers Inc.,  
N.Y., 1961, relied on p. 239.

OTHER REFERENCES

CHARLES N. LOVELL, Primary Examiner.